

1

2,775,504

**METHOD OF REMOVING HAIR AND WOOL FROM ANIMAL HIDES AND SKINS**

Haskiel Zalcman, Braybrook, Victoria, Australia

No Drawing. Application April 14, 1951,  
Serial No. 221,115

Claims priority, application Australia October 18, 1949

6 Claims. (Cl. 8—94.16)

This invention relates to the dehairing or removal of hair or wool from animal skins using the painting process wherein a paint composition is applied to the flesh side of the skin so that direct contact with the hair or wool is avoided so far as is practicable.

The invention is also particularly though not exclusively concerned with the removal of wool from sheepskins.

In the known or existing "painting" processes for dehairing or de-wooling skins, it is customary to brush or spray the flesh side of the skin with a "Paint" consisting of a mixture of sodium sulphide ( $Na_2S$ ) and/or sodium hydrosulphide ( $NaHS$ ) and lime ( $CaO$ ) in water in the desired concentration with or without an inert filler to produce the required consistency.

The presence of sodium salts in such "paints" results in a relatively high pH value which causes appreciable damage to the hide substance in the pelt or skin and to the wool or hair. Moreover in addition to the actual destruction of hide substance caused by the high pH value, the reaction between sodium ions and hide substance in such "paints" at pH values above 10.0 results in plumping or swelling of the pelt or skin which is the cause of further permanent damage. Plumping also has an adverse effect on depilation because it constricts the opening of the hair or wool follicle so that even though the root is sufficiently loosened it cannot be readily pulled unless the bulk of the root is pulped by more drastic chemical action.

For a considerable time it has been generally recognized that whenever sodium sulphide ( $Na_2S$ ) or sodium hydrosulphide ( $NaHS$ ) is used as a basic constituent in a "paint," damage to the skins and where the skin is a sheepskin to the wool as well is unavoidable. Wool so pulled is not to be compared with virgin wool, the wool fibers becoming harsh and reduced in tensile strength and elasticity. They are thickened so that a wool of for instance a 58 count is reduced in count to approximately 56. The reduction in tensile strength results in a lower tear in top-making and the wool is discolored and will not dye evenly. As a result of this damage the wool is invariably graded into a lower grade than virgin wool of the same fineness and character.

The object of the present invention is to achieve satisfactory depilation at a pH so far below the effective minimum in the prior art as to reduce damage in the pelt or hair or wool to a negligible quantity. This is achieved by—

(a) Eliminating the cause of excessive plumping and so avoiding the adverse binding effect on the hair or wool root.

(b) By increasing the hydrosulphide ion concentration and

(c) By controlling the pH down to the minimum value necessary for depilation having regard to the depilation load being kept to a minimum and the hydrosulphide ion concentration being increased to an economic maximum.

These objectives are attained broadly by using a paint

2

that is substantially devoid of sources of monovalent metal ions and which is maintained at a pH of less than about 12. The paint contains in addition to water a source of hydroxyl ions, a source of sulphide or hydro-sulphide ions; and may contain a buffer substance for controlling or repressing the hydroxyl ion concentration of the paint, thereby to continuously maintain the paint at relatively low pH as compared with paints now commonly used.

10 These objectives are attained more specifically, and preferably, by selecting as the unhauling accelerator calcium hydrosulphide ( $Ca(HS)_2$ ) which by reason of its property of depressing pH while not causing any plumping beyond that caused by lime alone enables the hydro-sulphide ion concentration to be heavily increased.

The paint composition preferably comprises calcium hydrosulphide ( $Ca(HS)_2$ ) and lime ( $CaO$ ) and water mixed in proportion, the concentration of calcium hydrosulphide ( $Ca(HS)_2$ ) being within the range of about 2% to about 30% and the concentration of lime ( $CaO$ ) being within the range of about 33% to about 1% each by weight of the composition to form a "paint" of suitable concentration for application to the skins; the consistency of the "paint" being adjusted as necessary by the addition of an inert filler. The inert filler may be, for example, kaolin.

The invention relates basically to the method of de-wooling sheepskins and dehauling skins which comprises applying to the flesh side of the skins a "paint" composition comprising calcium hydrosulphide ( $Ca(HS)_2$ ) and lime ( $CaO$ ) and water mixed in proportion, the concentration of calcium hydrosulphide ( $Ca(HS)_2$ ) being within the range of about 2% to about 30% and the concentration of lime ( $CaO$ ) being within the range of about 33% to about 1% each by weight of the composition the consistency of the "paint" being adjusted as necessary by the addition of an inert filler; allowing the "paint" composition to remain on the skins for a selected period of time; and subsequently pulling the loosened wool and hair from the skins.

The paint preferably used in the practice of my improved method is a composition comprising calcium hydrosulphide ( $Ca(HS)_2$ ) and lime ( $CaO$ ) and water mixed in proportion the concentration of calcium hydrosulphide ( $Ca(HS)_2$ ) being within the range of about 3% to about 10% and the concentration of lime ( $CaO$ ) being within the range of about 28% to about 4% each by weight of the composition to form a "paint" of suitable concentration for application to the skins the consistency of the "paint" being adjusted as necessary by the addition of an inert filler. It will be understood that the invention also provides the method of de-wooling sheepskins and dehauling skins, as hereinbefore described but using the last mentioned composition.

55 The composition is prepared simply by mixing the calcium hydrosulphide ( $Ca(HS)_2$ ) and lime ( $CaO$ ) and water in proportion, with or without the inert filler as is necessary for the adjustment of the consistency of the compositions, to obtain "paints" of suitable concentration for application to the skins; as explained herein-after.

The "paint" is applied to the skin by brushing or spraying on to the flesh side of the latter, which is then left for a predetermined period before the hair or wool is subjected to the pulling or other removing operation. Generally, the composition is of such concentration, with relation to the nature of the skin as hereinafter more fully explained, that it achieves its object in accordance with the invention, within about 24 hours after application to the skins.

In the treatment of skins other than sheepskins and hides, the period of depilation is lengthened as necessary.

according to the thickness, type and condition of the skin or hide to be treated.

In the prior art it was generally accepted that depilation was for practical purposes impossible at a pH lower than 12.3—12.5 which view led to the conviction that depilation by painting with a composition containing a high concentration of calcium hydrosulphide ( $\text{Ca}(\text{HS})_2$ ) was quite impossible by reason of the progressive reduction in pH as shown by the following table based on the applicant's work—

EFFECT OF CALCIUM HYDROSULPHIDE ( $\text{Ca}(\text{HS})_2$ ) ON THE pH OF CALCIUM HYDROXIDE ( $\text{Ca}(\text{OH})_2$ ) SUSPENSIONS

| Grams ( $\text{Ca}(\text{HS})_2$ )<br>per 100 grams liquor | pH    | Grams ( $\text{Ca}(\text{HS})_2$ )<br>per 100 grams liquor | pH    |
|------------------------------------------------------------|-------|------------------------------------------------------------|-------|
| 0.0                                                        | 12.61 | 8.0                                                        | 11.69 |
| 1.0                                                        | 12.26 | 9.0                                                        | 11.66 |
| 2.0                                                        | 12.07 | 10.0                                                       | 11.64 |
| 3.0                                                        | 11.95 | 12.5                                                       | 11.55 |
| 4.0                                                        | 11.86 | 15.0                                                       | 11.44 |
| 5.0                                                        | 11.80 | 20.0                                                       | 11.15 |
| 6.0                                                        | 11.76 | 25.0                                                       | 10.62 |
| 7.0                                                        | 11.72 | 30.0                                                       | 9.9   |

But it has been found by experiment by the applicant that effective depilation of sheepskins can be achieved by painting with a concentration of calcium hydrosulphide ( $\text{Ca}(\text{HS})_2$ ) as high as 30% by weight of the composition with the resultant pH as low as 9.9. At this concentration it was found to be unnecessary to provide more lime ( $\text{CaO}$ ) than 1% by weight of the composition. For economic reasons such a high concentration of calcium hydrosulphide ( $\text{Ca}(\text{HS})_2$ ) can be regarded as extreme and only significant as indicating the lower limits of hydroxyl ion concentration at which depilation is possible.

Further experiments demonstrated that with a concentration of calcium hydrosulphide ( $\text{Ca}(\text{HS})_2$ ), as low as 2% by weight of the composition could be used if the proportion of lime ( $\text{CaO}$ ) were increased to 33% by weight of the composition.

The results of the last mentioned experiment indicated that the pH (in this case 12.07) was higher than the optimum because the wool though much superior to wool removed by the sodium sulphide process was damaged to some extent.

Within these two extremes it has been found in practice that it is preferable to observe the following narrow limits according to the kind and type and condition of the skin and particular working conditions.

Calcium hydrosulphide ( $\text{Ca}(\text{HS})_2$ )—about 3% to about 10%.  
Lime ( $\text{CaO}$ )—about 28% to about 4%.

The experiments above referred to and the relative proportions of calcium hydrosulphide ( $\text{Ca}(\text{HS})_2$ ) and lime ( $\text{CaO}$ ) used bring out a number of factors, the significance of which appear not to have been appreciated in the prior art. Without a proper appreciation of them it was almost inevitable that it would be assumed, as was done, that satisfactory depilation with high concentrations of calcium hydrosulphide ( $\text{Ca}(\text{HS})_2$ ), or equivalent sources of hydrosulphide ions, is impracticable.

The factors referred to are:

1. That the plumping or swelling of a skin resulting from the presence of substantial quantities of monovalent cations in the conventional sources of hydrosulphide anions, that is, sodium sulphide ( $\text{Na}_2\text{S}$ ) and sodium hydrosulphide ( $\text{NaHS}$ ), required a pH value high enough to pulp the bulk of the hair or wool root, due to the fact that the follicle of the root was constricted by the plumping action;

2. That if a source of hydrosulphide anions associated with polyvalent cations is used a very much lower pH value would loosen the hair or wool root sufficiently to enable it to be removed since the plumping action is substantially eliminated;

3. That despite the facts that the depressing of the pH value of a lime suspension, as by the presence of calcium ions, is caused by the depressing of the solubility of the lime ( $\text{CaO}$ ) or other source of hydroxyl ions, and that hydroxyl ions react by combination with collagen and saponification of fat in a skin thus involving a reduction of hydroxyl ion concentration available to react on the keratin of the hair or wool root, it is still possible to bring sufficient additional lime ( $\text{CaO}$ ) or other source of hydroxyl ions into solution to replenish the loss of hydroxyl ion concentration even where the pH of the composition when applied is as low as 9.9. This is to be explained by the following further factors;

4. That the loss of hydroxyl ions due to reaction with collagen and fat varies with the concentration of the hydroxyl ions at various pH values, and appears to be relatively insignificant at low pH values as compared with that at high pH values. This would appear to follow from the fact that the concentration of hydroxyl ions at a pH of 11 is only one-tenth of that at a pH of 12, and one-twentieth of that at a pH of 12.3;

5. That at any given solubility of lime the rate at which undissolved calcium hydroxide ( $\text{Ca}(\text{OH})_2$ ) in a composition can be brought into solution, can be increased by increasing its bulk, and, therefore, the surface of it exposed to solution.

Having regard to the last two foregoing factors, it has been found that a proportion of 1% lime ( $\text{CaO}$ ) provides a sufficient surface of undissolved or unhydrolyzed hydroxide ( $\text{Ca}(\text{OH})_2$ ) to provide the necessary replenishment of hydroxyl ions at a pH of 9.9, and that at a pH of 12.15 a considerably larger proportion of lime ( $\text{CaO}$ ) is required.

It has been found by experiments that it is necessary to take into account both the rate of solubility as determined by the concentration of calcium ions and the rate at which the undissolved calcium hydroxide ( $\text{Ca}(\text{OH})_2$ ) at any given concentration of calcium ions can be brought into solution. Each of these factors must be taken into account according to the anticipated loss of hydroxyl ions.

If the skin to be treated is a thick and/or fatty skin increasing the surface of undissolved calcium hydroxide ( $\text{Ca}(\text{OH})_2$ ) exposed to solution may not be sufficient without reducing the proportion of calcium hydrosulphide ( $\text{Ca}(\text{HS})_2$ ) so as to reduce the depressing effect of the calcium ion concentration on the rate of solubility.

Experience has led the applicant to believe that it is desirable in some instances to limit the proportion of lime ( $\text{CaO}$ ) and therefore the surface of lime ( $\text{CaO}$ ) exposed to solution to that which is no more than sufficient to overtake towards the end of the selected period of skin treatment, the loss of hydroxyl ions due to reaction. If the proportion of lime ( $\text{CaO}$ ) is not so limited depilation will still be achieved but both the skin and the wool will suffer some damage indicating that the hydroxyl ion concentration at its full strength reacts for too long a period on the skin and wool roots. Hence the desirability, if the best results are to be secured where adjustment of consistency of a paint is called for, for the addition of an inert filler.

These problems of control have no such significance where the unhauling composition is brought into direct contact with the hair at its roots by immersion. There the maintenance of the pH at the hair roots is only slightly affected by loss of hydroxyl ions and the question of varying conditions of thickness and fattiness in the skin and the low rate of solubility of lime ( $\text{CaO}$ ), present no problem so far as depilation is concerned.

#### 70 PRACTICAL EXAMPLES OF TREATMENT

##### Example 1

A sheepskin with a wool count of 58 after being washed, soaked and deburred was painted with a "paint" containing—

## 5

About 7% calcium hydrosulphide ( $\text{Ca}(\text{HS})_2$ )  
 About 14% lime ( $\text{CaO}$ )  
 About 6% kaolin  
 About 73% water.

After painting the skin was folded in the middle and hung over a wooden pole for a period of 24 hours. The wool was then removed from the skin. Upon inspection it was found that the wool had a quality superior to that obtainable by treating a similar skin according to the practices hitherto followed in the art, whilst the skin likewise was in a superior condition.

The skin treated in the above example was of average condition, i. e., characterized by that degree of thickness and fat content associated with the skin of a sheep grown under average conditions as to rainfall in a locality suitable for the growing of wool of 58 count. The skin of a sheep grown under drought conditions, is less thick and carries less fat than the average and conversely a sheep grown under conditions of heavy rainfall and over-abundant feed is thicker and carries more fat than the average.

Sheepskins vary as to thickness and fat content according to type as well as condition and for a similar reason. Classified as to type according to the count of wool they carry skins carrying wool of higher counts are less thick and fatty than skins carrying wool of lower counts for the reason that fine wools are grown in drier areas than are coarse wools. But this variation is not very material in the case of skins carrying wool of counts above 58 first because the variation is relatively slight and next because it is offset by the occurrence of folds in the skins of sheep carrying fine wools or what is described as a "ribby" condition in its skin.

The composition used in the above example was found by trial to be that most suited to the treatment of skins of the type (expressed in terms of wool count) of a 56-58 count and of average condition. Taking this composition as a norm the operator should increase the proportion of calcium hydrosulphide ( $\text{Ca}(\text{HS})_2$ ) and decrease that of lime ( $\text{CaO}$ ) where the skins have the characteristic of a lesser thickness and fat content than a skin of 56-58 wool count of average condition whether that characteristic is due to variation in type or condition or both. Conversely, where the skins to be treated are characterized by greater thickness and fat content the operator should decrease the proportion of calcium hydrosulphide and increase that of lime.

## Example 2

As an illustration of adjustments which should be made, the example of a sheepskin of average condition and having a wool count of 50 may be quoted. A skin of this type and condition after being washed, soaked and deburred was painted with a "paint" containing

About 3% calcium hydrosulphide ( $\text{Ca}(\text{HS})_2$ )  
 About 25% lime ( $\text{CaO}$ )  
 About 71% water.

After painting the skin was folded in the middle and hung over a wooden pole for a period of 24 hours. The wool was then removed from the skin. As in the case of the previous example it was found on inspection that both the wool and the skin were of superior quality and condition to what was obtainable by treating a similar skin according to the practices hitherto followed in the art.

As previously indicated skins carrying wool of higher counts than 58 do not by reason of their type alone call for any considerable variation in the proportions of calcium hydrosulphide ( $\text{Ca}(\text{HS})_2$ ) and lime ( $\text{CaO}$ ). Since these skins are most frequently characterized by a "ribby" condition it is found in practice that the composition as described in the first example is ordinarily the most suited to their treatment. For practical purposes skins of this type may be treated in the same manner as skins of the

## 6

type of a wool count of 56-58 with similar variations according to condition.

With every skin of whatever type or condition it is necessary to apply a "paint" of lower calcium hydrosulphide ( $\text{Ca}(\text{HS})_2$ ) concentration and higher lime ( $\text{CaO}$ ) concentration to the neck and butt portions of the skin where the skin is thicker than it is elsewhere. As an indication of the adjustment here called for it may be taken that where a paint as in Example 1 above is suitable for the main part of the skin a paint as in Example 2 would be used on the neck and butt.

The proportions in all the above examples are adjusted to a period of depilation of about 24 hours at normal room temperature, say 70° or 80° F. This period is 15 normal practice in the fellmongering art and the fact that it is so, operates very much to the disadvantage of the users of paints hitherto used in the art. Operating at a high pH, as has been so in the past, it is impossible to leave skins painted over a weekend without seriously increasing the damage to both skin and wool. This further damage is either accepted or the wool is pulled during the weekend at increased labor cost. By the practice of this invention skins may be left over a weekend before pulling without serious increase in damage to either the skin or 20 wool.

The treatment of hides and skins other than sheepskins follows the same principles, but the period of depilation varies from 24 hours to 96 hours or even longer according to the thickness type and condition of 25 the skin or hide to be treated.

A salted calfskin of approximate weight 5 lbs. green was washed and soaked for about 12 hours and then fleshed and painted with a "paint" containing,

35 About 5% calcium hydrosulphide ( $\text{Ca}(\text{HS})_2$ )  
 About 7% lime ( $\text{CaO}$ )  
 About 88% water.

After painting the skin was folded in the middle and laid on a barrow for a period of 24 hours.

40 The skin was then dehaired in a skudding machine and it was found that the hair was in a good condition and the skin was in good condition.

The best results are achieved particularly with sheepskins characterized by thickness and excessive fat by previous soaking and the action of machine deburring also contributes to more effective depilation at a minimum pH. Though soaking of the skin is not essential it is found that after soaking the proportion of ( $\text{Ca}(\text{HS})_2$ ) may be increased and the pH of the composition consequentially 45 decreased beyond what is necessary where there is no previous soaking.

Although calcium hydrosulphide and lime in the proportions indicated have been found highly satisfactory in practice, there are other substances and modifications of 50 the process that may be used to obtain the desired results. The first requirement is that the paint be devoid, or substantially devoid, of sources of monovalent metal ions, and this is true whether calcium hydrosulphide is used, or some equivalent substance. The substantial elimination of the sources of monovalent metal ions substantially avoids plumping or swelling of the skin, and thereby makes possible the use of lower pH solutions for the 55 depilation of the wool or hair. This concept itself is of great importance in the practice of the invention.

60 Broadly speaking, the invention contemplates a composition substantially devoid of sources of monovalent metal ions, and comprising any suitable polyvalent metal source of hydroxyl ions, as hereinafter defined a suitable source of sulphide or hydrosulphide ions, and, where necessary, a buffer material for controlling the hydroxyl ion concentration in the composition, so that the composition has a pH value of about 12 or less. Although lime is obviously the most practical source of hydroxyl ions, other suitable bases such for example as barium hydroxide ( $\text{Ba}(\text{OH})_2$ ) or strontium hydroxide ( $\text{Sr}(\text{OH})_2$ ) might 65

also be used, and possibly also magnesium hydroxide ( $Mg(OH)_2$ ).

The hydrosulphide ion which must be present in suitable quantities to effect depilation may be provided in various ways. The most effective source is calcium hydrosulphide which should be in the proportion of 2 to 30% in order to maintain the pH of the solution below about 12.

Instead of mixing calcium hydrosulphide with lime, the hydrosulphide ions may be provided by passing hydrogen sulphide ( $H_2S$ ) into a slurry of lime in water, thereby forming a mixture of calcium hydrosulphide and unchanged lime. Or, the hydrogen sulphide could be passed into a slurry of lime and calcium sulphide, in which case the hydrogen sulphide would be absorbed and the pH of the solution lowered.

Instead of using a calcium salt as a base for the hydrosulphide ion, other metal sulphides may be used so long as the metal is not monovalent and the metal sulphide is appreciably soluble in lime water, or, if not soluble, then if the hydroxide of that metal is even more insoluble in water, so that the metal sulphide will act with calcium hydroxide to form calcium sulphide or hydrosulphide and an insoluble metal hydroxide.

Accordingly, sulphides of barium, strontium, magnesium, and aluminum may be used satisfactorily, although in some instances of high solubility a buffer material would have to be used in order to control the pH to below about 12, such buffer being a suitable acid or soluble calcium salt.

Calcium chloride or a soluble calcium salt may be used as a control by providing calcium ions which repress the solubility of the calcium hydroxide to thereby maintain the desired pH value of about 12 or less.

Instead of using a soluble calcium salt a suitable acid may be used provided such acid produces a calcium salt that is at least moderately soluble. Thus, hydrochloric acid, acetic acid, hydrobromic acid, formic acid, lactic acid, nitric acid, nitrous acid, tartaric acid, and citric acid, are common acids whose calcium salts are soluble, and which would normally provide the soluble calcium salt needed to repress the solubility of calcium hydroxide.

Even some sulphides that would normally be deemed ineffective in a lime solution, because they form insoluble sulphides, may be made effective if used with some added substance that would cause them to dissolve. All that appears to be necessary is that the sources of monovalent cations are substantially avoided, that there be a suitable source of hydroxyl and hydrosulphide ions, and that the pH is properly controlled by buffer substances when necessary to a value of about 12 or less.

In this specification and the following claims the word "paint" has the meaning understood by those skilled in the art of de-wooling sheepskins and dehairing skins; the expression "suitable concentration" means the relative concentration of calcium hydrosulphide ( $Ca(HS)_2$ ) and lime ( $CaO$ ) found to achieve depilation within a given period with the most favorable results as regards the skins and in the case of sheepskins the wool as well having regard to the thickness and fat content of the skins; and, the expression "inert filler" means a finely divided substance the primary purpose of which as an additive to the composition is to thicken the consistency of the composition.

While I have described particular embodiments of my invention, it will occur to those skilled in the art that various changes, modifications and equivalents may be made or used without departing from my invention, and I, therefore, intend, in the appended claims, to cover all such changes, modifications and equivalents as fall within the true spirit and scope of my invention.

This application is a continuation in part of my earlier application Serial No. 180,897, filed August 22, 1950, now abandoned.

I claim:

1. In the art of depilating lamb and sheep skins by applying a depilatory paint to the flesh side of the skins, the method of effecting depilation to obtain high quality wool while preserving the quality of the skin which consists in applying to the flesh side of the skin an aqueous composition which is substantially free of sources of monovalent metal cations and which comprises calcium hydrosulphide and lime, the calcium hydrosulphide being about 3 to 7% and the lime about 25 to 14%, each by weight of the composition, the proportion of calcium hydrosulphide decreasing and of lime increasing within the above ranges with the increasing thickness and fat content of the skin, the composition having a pH of not more than 12 and not less than about 11.7, and the source of hydroxyl ions being sufficient in quantity to provide an undissolved reserve thereof suspended in the composition; allowing the composition to remain on the skin until the wool is loosened, and then pulling the loosened wool from the skin.
2. In the art of depilating lamb and sheep skins by applying a depilatory paint to the flesh side of the skins, the method of effecting depilation to obtain high quality wool while preserving the quality of the skin which consists in applying to the flesh side of the skin an aqueous composition which is substantially free of sources of monovalent metal cations and which comprises calcium hydrosulphide and lime, the calcium hydrosulphide being about 3 to 7% and the lime about 25 to 14%, each by weight of the composition, the calcium hydrosulphide decreasing toward 3% and the lime increasing toward 25% to provide a lower ratio of calcium hydrosulphide to lime when the composition is applied to the neck and butt portions of the skin as compared with the ratio of calcium hydrosulphide and lime in the composition applied to other portions of the skin, whereby the proportion of calcium hydrosulphide decreases and of lime increases with the increasing thickness and fat content of the skin, the composition having a pH of not more than 12 and not less than about 11.7, and the source of hydroxyl ions being sufficient in quantity to provide an undissolved reserve thereof suspended in the composition; and allowing the composition to remain on the skin until the wool is loosened.
3. In the art of depilating lamb and sheep skins by applying a depilatory paint to the flesh side of the skins, the method of effecting depilation to obtain high quality wool while preserving the quality of the skin which consists in applying to the flesh side of the skin an aqueous composition which is substantially free of sources of monovalent metal cations and which comprises calcium hydrosulphide and lime, the calcium hydrosulphide being about 3 to 10% and the lime about 28 to 4%, each by weight of the composition, the proportion of calcium hydrosulphide decreasing and of lime increasing within the above ranges with the increasing thickness and fat content of the skin, composition having a pH of not more than 12 and not less than about 11.6, and the source of hydroxyl ions being sufficient in quantity to provide an undissolved reserve thereof suspended in the composition; allowing the composition to remain on the skin until the wool is loosened, and then pulling the loosened wool from the skin.
4. In the art of depilating lamb and sheep skins by applying a depilatory paint to the flesh side of the skins, the method of effecting depilation to obtain high quality wool while preserving the quality of the skin which consists in applying to the flesh side of the skin an aqueous composition which is substantially free of sources of monovalent metal cations and which comprises calcium hydrosulphide and lime, the calcium hydrosulphide being about 3 to 10% and the lime about 28 to 4%, each by weight of the composition, the calcium hydrosulphide decreasing toward 3% and the lime increasing toward 28% to provide a lower ratio of calcium hydrosulphide to lime

when the composition is applied to the neck and butt portions of the skin as compared with the ratio of calcium hydrosulphide and lime in the composition applied to other portions of the skin whereby the proportion of calcium hydrosulphide decreases and of lime increases with the increasing thickness and fat content of the skin, the composition having a pH of not more than 12 and not less than about 11.6, and the source of hydroxyl ions being sufficient in quantity to provide an undissolved reserve thereof suspended in the composition; and allowing the composition to remain on the skin until the wool is loosened.

5. In the art of depilating sheep skins, the method as set forth in claim 1 in which the aqueous composition includes an inert filler in such quantity as to give the 15 composition the consistency required for application and adherence to the flesh side of the skins.

6. In the art of depilating lamb and sheep skins by applying a depilatory paint to the flesh side of the skins, the method of effecting depilation to obtain high quality wool while preserving the quality of the skin which consists in applying to the flesh side of the skin an aqueous composition which is substantially free of sources of monovalent metal cations and which comprises calcium hydrosulphide and lime, the calcium hydrosulphide being about 3% to 30% and the lime about 33% to 4%, each by weight of the composition, with the lime being at least 7% when the calcium hydrosulphide concentration is at about 3%, the proportion of calcium hydrosulphide decreasing and of lime increasing within the above ranges with the increasing thickness and fat content of the skin, the composition having a pH of not more than 12 and not less

than about 9.9, and the source of hydroxyl ions being sufficient in quantity to provide an undissolved reserve thereof suspended in the composition; allowing the composition to remain on the skin until the wool is loosened, 5 and then pulling the loosened wool from the skin.

#### References Cited in the file of this patent

#### UNITED STATES PATENTS

|    |           |        |                |
|----|-----------|--------|----------------|
| 10 | Re. 4,549 | Siebel | Sept. 12, 1871 |
|    | 1,041,897 | Stone  | Oct. 22, 1912  |
|    | 2,169,148 | Jaeger | Aug. 8, 1939   |
|    | 2,487,558 | Kamlet | Nov. 8, 1949   |

#### OTHER REFERENCES

Thies et al.: article in J. A. L. C. A., vol. 37, 1942, pages 93-102.

"Progress in Leather Science 1920-1945," pages 176, 118 and 189, pub. 1948 by Printing Craft Ltd., Mansfield, England.

20 Moore, in J. A. L. C. A., vol. 22, 1933, pages 206-216.

"Tanning Processes," by Orthmann, publ. 1945 by Hide and Lea. Publ. Co., pages 1, 2, 40 and 41. (Copy P. O. S. L.)

25 "Progress in Leather Science 1920-1945," page 188, publ. 1948 by Printing Craft, Mansfield.

"Circular to Fellmongers No. 8," 3 p., September 1949, pub. by Commonwealth Scientific & Ind. Res. Or. Div. of Ind. Chem., Melbourne, Australia.

30 Bowes et al.: B. L. M. R. A. Lab. Report No. 25, part V, 1946, 8 pages.